

## UNITED STATES PATENT OFFICE

CHARLES D. RUSSELL, OF SHEBOYGAN, WISCONSIN, ASSIGNOR TO RUSELITE CORPORATION, OF MILWAUKEE, WISCONSIN, A CORPORATION OF WISCONSIN

## ART OF METALLURGY

No Drawing.

Application filed July 21, 1930. Serial No. 469,640.

This invention relates to improvements in the art of metallurgy, and more specifically to an alloy and mode of producing the same.

It is one of the objects of this invention to provide an improved alloy which possesses the desirable characteristics of high tensile strength, tenacity, and ductility, and which may be cast or worked with or without the necessity of additional heat treatment to bring out the above mentioned properties.

A further object of this invention is to provide an improved alloy which may be readily polished and which is resistant to corrosion.

A further object of this invention is to provide an improved alloy, which, when cast, can be bent and twisted while cold.

A further object of this invention is to provide an improved alloy which possesses a high electrical resistance.

20 A further object of this invention is to produce an alloy which is particularly adapted for use in highly stressable springs or the like.

With the above and other objects in view, 25 the invention consists of the improved alloy and mode of producing the same, and all its parts and combinations, as set forth in the claims, and all equivalents thereof.

The improved alloy, in its preferred form, 30 comprises a major portion of copper, together with aluminum, molybdenum and tantalum, the molybdenum serving as a strengthener and the tantalum serving to render the alloy resistant to corrosion and of high electrical resistance. In some instances, other 35 corrosion resistant material such as chromium may be substituted for tantalum. The following tabulation discloses one combination of ingredients together with a desirable 40 range of proportions for each of said ingredients.

|                    | Per cent |
|--------------------|----------|
| Copper-----        | 85 -95   |
| Aluminum-----      | 3 -12    |
| 45 Molybdenum----- | .10- 5   |
| Tantalum-----      | .10- 3   |

In forming the alloy, the copper and aluminum may be mixed together and heated to a 50 temperature of approximately 2300 degrees

Fahrenheit, a suitable flux being utilized. Next molybdenum and tantalum may be added together, and the resulting mixture may be reduced in 25 to 30 minutes. The molten mass is kept at a bright red heat at all times and is stirred well before being poured into molds.

By utilizing the above method, and the ingredients recited in the range of proportions set forth in the formula, a bronze alloy is formed which is of exceptionally high tensile strength and which possesses unusual ductility for an alloy of such strength. The material produced is also extremely resistant to corrosion and is therefore capable of advantageous use for many purposes, such as for steam turbine blading, springs, and the like. The alloy can be employed for castings of all kinds, and for drawing, rolling and forging.

## What I claim is:

1. An alloy comprising a major portion of copper together with 3-12% aluminum, .10-5% molybdenum, and .10-3% tantalum, said alloy possessing high tensile strength, 75 tenacity, and ductility.

2. An alloy comprising approximately 90% copper, 7% aluminum, 2% molybdenum, and 1% tantalum, said alloy possessing high tensile strength, tenacity, and ductility.

3. An alloy comprising a major portion of copper together with 3-12% aluminum, .10-5% molybdenum, and .10-3% of one of the corrosion resisting metallic elements tantalum and chromium, said alloy possessing 85 high tensile strength, tenacity, and ductility.

In testimony whereof I affix my signature.

CHARLES D. RUSSELL.